

# UNITED STATES PATENT OFFICE.

JACOB EISELSTEIN, OF EGG HARBOR CITY, NEW JERSEY.

## PROCESS OF MANUFACTURING AND FINISHING PARCHMENT-PAPER.

SPECIFICATION forming part of Letters Patent No. 621,603, dated March 21, 1899.

Application filed August 25, 1898. Serial No. 689,453. (No specimens.)

*To all whom it may concern:*

Be it known that I, JACOB EISELSTEIN, a citizen of the United States, residing at Egg Harbor City, in the county of Atlantic, State 5 of New Jersey, have invented a new and useful Improvement in Processes of Manufacturing and Finishing Parchment-Paper, which improvement is fully set forth in the following specification.

10 My invention consists of an improved process of manufacturing and finishing parchment-paper whereby I am enabled to produce a superior article and one which has marked advantages over the parchment-papers now 15 in the market. To this end I first parchmentize the paper in the usual manner, and after the same has been washed I pass it through a heated solution or bath composed of certain ingredients, to be hereinafter referred to in detail, the function of which is 20 to fill the pin-holes in the paper and to give body thereto. The paper after passing through the solution or bath above referred to is run upon a drier, and from there it is 25 conducted over a friction-calender or a super-calender and submitted to another bath or solution while passing over the hot roll on the calender. The elements of the last-mentioned bath serve to give a gloss to the paper and to 30 make the same transparent and in addition to keep the paper soft, so it will not become brittle in passing through the calender, the finished product being soft, glazed, and highly finished, which excellent properties it will 35 retain indefinitely.

The invention further consists of novel details in the process of manufacture, all as will be hereinafter fully set forth, and particularly pointed out in the claims.

40 In carrying out my invention I take paper which is parchmentized in the usual manner, and the same after being washed is passed through a heated solution or bath composed of dextrine, china-clay, glucose, and water, 45 the same being taken in substantially the following proportions: ten per cent. dextrine, ten per cent. china-clay, ten per cent. glucose, and seventy per cent. water. The china-clay and glucose are to be well mixed before 50 being placed in the water, and the foregoing so-

lution or bath must be hot, so that the paper will not be chilled before being run over the drier. The function of the dextrine and china-clay is to fill pin-holes in the paper, while the object of the employment of the 55 glucose is to give body to said paper. After the paper has been passed through the above-named bath it is run over the drier and then over a friction-calender or a supercalender and treated to a solution of wax or paraffin, 60 silicate of soda, talc, oil, and glycerin while passing over the hot roll on the calender, the above ingredients being combined substantially as follows: five percent. wax or paraffin, ten per cent. silicate of soda, ten per cent. 65 talc, ten per cent. oil, and sixty-five per cent. glycerin. The above solution is applied to the paper in any suitable manner, preferably by a woolen-cloth spreader or brush to distribute the same evenly on the roll, where it 70 is forced into the paper by the heat of the roll over which the paper is passed. The paper is then turned and again passed through the calender to be treated on the other side thereof to the same solution—viz., wax or 75 paraffin, silicate of soda, talc, oil, and glycerin, combined substantially as above specified. In the last solution the wax or paraffin and silicate of soda give a gloss to the paper, while the function of the oil is to make the paper 80 transparent, the talc to economize on glycerin, and the object of the glycerin is to keep the paper soft, so it will not become brittle in passing through the calender, the paper when treated and finished in the manner 85 above described becoming soft, glazed, and highly finished, which excellent properties are retained indefinitely. It will be apparent that by the foregoing steps a simple and expeditious process is attained, whereby paper 90 thus treated is greatly superior to parchment-paper produced in accordance with the usual process of manufacture.

Having thus described my invention, what I claim as new, and desire to secure by Letters 95 Patent, is—

1. The herein-described process of treating paper which consists in passing the same first through a hot bath of dextrine, china-clay, glucose and water, and next treating said 100

paper with a solution of wax or paraffin, silicate of soda, talc, oil and glycerin.

2. The process of treating paper which consists of parchmentizing the same, washing 5 said paper, passing the latter through a heated solution of dextrine, china-clay, glucose and water, running the paper upon a drier and

thence over a calender and lastly treating said paper to a solution composed of wax or paraffin, silicate of soda, talc, oil and glycerin. 10

JACOB EISELSTEIN.

Witnesses:

ROBT. A. MEIER,  
JOHN A. WIEDERSHEIM.